

Patented Oct. 14, 1952

2,613,579

## UNITED STATES PATENT OFFICE

2,613,579

## SIZING AND BLEACHING A WET WEB

Robert L. McEwen, Williamsville, N. Y., assignor  
to Buffalo Electro-Chemical Company, Inc.,  
Tonawanda, N. Y.

No Drawing. Application August 27, 1947,  
Serial No. 770,955

3 Claims. (Cl. 93—102/162-12)

1

The present invention relates to the manufacture of a sized, bleached, paper sheet and more particularly to a method of manufacturing such a sheet wherein the sizing and bleaching operation proceed substantially concurrently.

Recent improvements in paper-making technology indicate that obtainment of better brightness of paper stock is probably best performed upon the paper-making machine, as contrasted to bleaching the pulp stock itself. Examples of this improved technique are described in Patent No. 2,150,926 granted on March 21, 1939 to Kauffmann and Wolfe, and in Patent No. 2,125,634 granted on August 2, 1938 to Heritage. These improvements in the brightening of paper show that brightened paper stock can be produced economically and with little change in the normal paper manufacturing procedure by applying the brightening or bleaching agent, preferably a peroxide, to the formed paper sheet while it is on the paper-making machine.

These suggestions generally indicate that best results in paper bleaching are obtained by application of the brightening agent to the consolidated paper sheet and subsequently removing moisture as, for instance, by passing the sheet over the drying element normally associated with the conventional paper-making machine.

However, in this type of operation, difficulty has been experienced in producing papers which are sized sufficiently or which are properly sized to resist moisture penetration and to retain a sharp printing impression or a sharp pen and ink impression without "feathering." Even where the normal quantities of usual or conventional size are present in the paper, the usual alkalies associated with the alkaline peroxide solution used upon the machine, to obtain bleached or brightened paper, appear to destroy the sizing properties of the material added for sizing purposes. Many attempts have been made to overcome this deficiency in sheets resulting from the machine bleaching with but indifferent success.

Thus, attempts have been made to increase the amount and type of sizing in the beater, yet it has been found that in either case, the alkaline peroxide solution will reduce the effectiveness of or destroy the sizing in the sheet to the depth to which the alkaline bleach liquor penetrates. Secondly, it has been attempted to first bleach the sheet with alkaline peroxide and thereafter add an amount of size sufficient to restore the desired degree of sizing required. However, a procedure of this type is not generally applicable to the various types and weights of paper as

2

additional drying capacity is required to remove the excess amount of moisture necessarily used to incorporate the sizing agent into the bleached sheet; moreover, most papers are of such light weight that the sheet structure is adversely affected and even destroyed upon application thereto of a sizing solution, resulting in production of unsalable paper stock. The decrease in the wet strength of the sheet produces an unduly large percentage of breakage. In some cases, so-called "curling" difficulties are found. A further disadvantage of first bleaching the paper sheet on the machine and subsequently sizing the bleached paper is that, in the employment of many of the conventional sizes, the paper has a tendency to revert in color by reason, possibly, of some chemical action between the residual chemicals from the bleaching solution and the added size. This is particularly noticeable in the employment of casein and also in the employment of a so-called alum wash, both usual sizing treatments.

The application of the sizing agent subsequent to the application of the bleach liquor, moreover, may result in a leaching out of the active bleaching ingredient from the impregnated sheet into the main body of the size solution, thereby resulting in bleaching inefficiency.

Reversing the procedure and applying the sizing in amounts considerably in excess of that normally employed, such as in the production of hard sized sheets, results in either the destruction of the size or the production of a paper which is substantially repellent to the bleaching solution, in which case the efficiency is reduced to such an extent that little or no bleaching occurs.

Where substantial amounts of wax emulsion are added to the beater as a sizing agent, it has been found that the quantity of wax solids necessary to produce a sized and machine bleached sheet is such that the paper properties are highly undesirable because the sheet is unctuous, floppy, and too soft, and the sheet, in many instances, is not receptive to ink. Where excessive quantities of wax are incorporated in the sheet, the sheet is then relatively repellent to the aqueous bleaching solution subsequently applied thereto.

The objects of the present invention are to overcome the many difficulties encountered heretofore in the production of machine bleached paper.

It is also an object to improve not only the brightness of machine bleached paper but also to improve the quality of sizing thereof.

It is also an object of the invention simultan-

ously to apply to a sheet of paper, upon a paper-making machine, both a sizing agent and a bleaching agent thus permitting production of bleached, sized paper at high production rates and where there is substantially no increase in steam costs for drying.

The invention permits the production of sheets satisfactorily surface-sized for printing and writing, from unsized or slack-sized sheets which may have been partially sized in the beater.

In accordance with the principles of the present invention, the alkaline peroxide solution and an inert wax size are added simultaneously to the formed sheet as it progresses through the machine. In general, the point of application of the mixture of alkaline peroxide and wax size will be one at which the moisture content of the formed paper is greater than about 10%. That is to say, at any convenient point in the travel of the sheet wherein the machine as used still retains sufficient drying capacity to dry the sheet to the desired moisture content as, for instance, at the smoothing press or in advance of or between a series of driers.

The novel feature of the invention resides particularly in the ability to bleach the paper sheet while simultaneously forming therein a controllable degree of water resistance. The treating emulsion of wax and peroxide is prepared from any suitable wax size as, for instance, the generally employed paraffin or microcrystalline wax in emulsion form and an alkaline peroxide. The resulting emulsion may contain any desired amount of wax solids as, for instance, from about 0.1 to several percent or more as, for instance, 5%. The choice of this concentration will, of necessity, be dictated by the amount of sizing agent to be employed upon the particular sheet and the weight of the sheet. In general, the amount of wax desired in the sheet will be that quantity sufficient to size the sheet to a degree where it will receive the ink, either in liquid or paste form, without "feathering," and to a degree insufficient to cause skipping or repellency of the previously described ink.

The following examples are given as merely illustrative of the principles of the invention and are not to be deemed limitative thereof as, obviously, there will be many variations in the weight of paper produced, the amount of size to be added to the paper and the degree of brightening desired, it being understood that the invention is applicable generally to the production of substantially all types of paper sheets.

#### Example I

A pulp stock was prepared from bleached sulfite pulp and unbleached mechanical or ground wood pulp, and paper was prepared from the pulp on a conventional Fourdrinier paper machine. The pulp stock had been treated in the beater with 1.25% rosin based on the weight of the dry pulp. The finished paper as discharged from the machine possessed a brightness of 49.5 as measured in the usual manner with a photoelectric colorimeter. The sheets so produced, although sized, would feather to ink to a slight degree.

#### Example II

The same stock as described in Example I was used in preparation of an additional portion of paper except that a bleaching solution containing hydrogen peroxide and trisodiumphosphate was applied to each face of the paper sheet immediately preceding the driers. The amount of the

bleach solution employed was such that 1.4% of hydrogen peroxide (100 volume basis), and 0.8% trisodiumphosphate, each based on the weight of bone dry paper, was applied. The dry calendered sheet discharging from the machine had a brightness of 58 units. Although the brightness of the sheet was increased 8.5 units, the brightened sheet feathered extremely badly and was of no value whatsoever from the ink reception standpoint.

#### Example III

The same pulp as described in Example I was used to produce an additional amount of paper which was treated with the amount and type of bleaching agent and alkali specified in Example II. However, there was mixed with the alkaline bleach solution sufficient emulsified wax so that, upon application of the bleach-wax size solution to the paper sheet, there was also applied to the sheet 0.25% wax solids based on the weight of bone dry paper.

As the mixed wax emulsion-alkaline peroxide solution was applied to the paper sheet while the latter still contained a substantial amount of water, that is in advance of the driers, both the wax and the peroxide were able to penetrate below the surface of the sheet and the resulting sheet was brightened 9.7 units above that of the untreated stock of Example I. The finished sheet was also sufficiently sized as, when tested with pen and ink, this sheet showed no feathering nor was any skipping of the ink apparent, the writing being continuous.

It will be understood that the amount of wax to be employed will be entirely dictated by the type of pulp used and the type of paper desired to be produced. However, in general, it has been found that in operating in accordance with the present invention, and applying wax size simultaneously with the alkaline peroxide to a slack sized sheet, in general, at least 0.1% wax solids should be applied to the sheet, based on the dry weight of the sheet. This lower limit will, of course, vary depending upon the amount of beater sizing in the sheet, the type of pulp employed, the operating speeds of the machinery, and the weight of the paper as, in some instances, 0.1% will be insufficient to size the sheet to pen and ink. The upper limit of the amount of wax will also vary but will generally be found to be in the neighborhood of  $\frac{1}{2}\%$  to 1% wax solids on a bone dry basis. Quantities in excess of this amount produce oversizing, greasiness or unctuousness through the paper with resultant floppy sheets, and too great an excess tends to produce a wax coating rather than a wax sizing.

The amount of peroxide to be employed will depend upon the previous history of the pulp, that is, whether the same be a bleached, purified pulp, or an unbleached, ground wood pulp, or mixtures of various types of pulp, and also upon the degree of bleaching desired in the finished paper product. The amount of hydrogen peroxide calculated as 100 volume hydrogen peroxide may vary from about 0.5% to 10% or even higher. The mixed peroxide wax emulsion may contain penetrants or wetting agents to aid in carrying the solution into the sheet as well as tinting agents, starches, etc. In addition to hydrogen peroxide, the solution should contain an alkali and preferably should be made alkaline with a phosphate such as trisodiumphosphate, sodiumpyrophosphate or the meta phosphates such as hexametaphosphate. It is found that

2,613,579

5

the usual alkalies employed with hydrogen peroxide are unsuited for the simultaneous bleaching and sizing of paper sheets, and best bleaching and sizing results are obtained by employing a phosphate as the primary alkali in conjunction with hydrogen peroxide.

The peroxide-wax emulsion is best prepared by adding the previously dispersed and diluted wax to the alkaline peroxide solution. The wax may be of any suitable type, such as paraffin wax or micro crystalline wax, prepared by well known emulsifying operations.

By addition of the wax-peroxide emulsion to the formed slack sized sheet prior to its entrance into the drier, a minimum amount of moisture need be removed from a sheet by the drier while, at the same time, the peroxide solution and the particles of wax are able to penetrate the sheet to the desired degree and to effect simultaneously the desired bleaching and the desired degree of sizing.

It will be noted that by the simultaneous application of the wax size and peroxide solution, 10 to 15% additional brightening action is obtained.

What is claimed is:

1. The method of sizing and bleaching a sheet of paper consisting in applying to a formed paper sheet containing at least about 10% moisture, an aqueous solution consisting essentially of hydrogen peroxide made alkaline with a phosphate of sodium and a dispersion of wax in amount to add about  $\frac{1}{10}$ % to 5% wax, and from 0.5% to 10% hydrogen peroxide based on the weight of dry paper and thereafter passing the so treated sheet over heated drying rolls to dry the same, whereby penetration of said wax below the surface of the paper will occur without causing the surface to be ink-resistant.

5

10

15

20

25

30

35

6

2. The method of sizing and bleaching a formed paper sheet which consists in applying to the sheet, while the same contains excess moisture, an aqueous solution consisting essentially of hydrogen peroxide made alkaline with a phosphate of sodium and a dispersion of wax in amount to add about  $\frac{1}{10}$ % to 5% wax, and from 0.5% to 10% hydrogen peroxide based on the weight of dry paper and thereafter drying the sheet.

3. The method of preparing a bleached, sized sheet of paper which consists in applying to a formed paper sheet, before said sheet has been fully dried, an aqueous composition consisting essentially of hydrogen peroxide made alkaline with a phosphate of sodium and a dispersion of wax and in amount to add about  $\frac{1}{10}$ % to 5% wax and 0.5% to 10% hydrogen peroxide based on the weight of dry paper, and thereafter drying the sheet at an elevated temperature whereby the same is bleached and properly sized for ink writing and printing.

ROBERT L. McEWEN.

#### REFERENCES CITED

The following references are of record in the file of this patent:

#### UNITED STATES PATENTS

| Number    | Name          | Date          |
|-----------|---------------|---------------|
| 52,788    | Gwynn         | Feb. 20, 1866 |
| 1,797,048 | Clapp         | Mar. 17, 1931 |
| 1,957,370 | Thomas        | May 1, 1934   |
| 2,020,328 | Rafton        | Nov. 12, 1935 |
| 2,125,634 | Heritage      | Aug. 2, 1938  |
| 2,150,926 | Kauffmann     | Mar. 21, 1939 |
| 2,510,595 | McEwen et al. | June 6, 1950  |